

## UNITED STATES PATENT OFFICE

2,506,695

## COMPOSITION OF MATTER

Zeno W. Wicks, Jr., New York, N. Y., assignor to  
 Interchemical Corporation, New York, N. Y., a  
 corporation of Ohio

No Drawing. Application September 11, 1947,  
 Serial No. 773,523

12 Claims. (Cl. 106—239)

1

This invention relates to compositions of matter especially adapted for use in dispersing pigments for incorporation into pigmented compositions such as paints, varnishes, lacquers, enamels, inks and the like.

In the manufacture of pigmented coating compositions it is frequent practice to first disperse the pigment in a vehicle to form a pigmented paste before incorporating it into the paint, varnish, lacquer, or ink vehicle. This dispersion of pigment in vehicle is generally accomplished by grinding the pigment and the appropriate amount of vehicle in a suitable mixer such as a pebble mill, ball mill, roller mill, or dough mixer, and the vehicle employed is commonly referred to as a grinding vehicle. Essential properties of these grinding vehicles are: compatibility with the vehicle into which they will be subsequently incorporated, low viscosity, good wetting properties, non-reactivity with pigments, paleness of color, should not discolor at relatively high baking schedules if the resulting coating is to be baked, should not show tackiness in an air-dried film, and should be free from skinning tendencies.

Due to the large variety of protective coating compositions that are manufactured and the necessarily large variety of vehicles used in formulating them, it has been necessary for the paint, varnish and lacquer manufacturers to keep in stock a large variety of pigment grinding vehicles—i. e. a grinding vehicle to be used with each type of paint, varnish and the like that is to be produced. For example, linseed oil has been used as a grinding vehicle for pigmenting pastes for oil base paints but these pastes cannot be used with alkyd resin or nitrocellulose formulations. Likewise, a varnish containing oil modified alkyd resins and linseed oil has been used as grinding vehicle for pigments for incorporation in alkyd base compositions but this vehicle cannot be used with oleoresinous or lacquer formulations.

The protective coating industry has long desired a vehicle which can be used to make pigment pastes that are compatible with all the types of vehicles used in formulating protective coatings, such as siccatives, oleoresinous varnishes, synthetic resin compositions, lacquers, etc. In addition to being compatible with the various vehicles used in formulating coating compositions, the grinding vehicle should possess the other desirable properties for grinding vehicles that are listed hereinabove. Accordingly, it is an object of the present invention to

2

produce grinding vehicles that can be used to make pigment pastes for incorporation into a large variety of coating composition vehicles. Other objects of the invention will become apparent as the description of the invention proceeds.

The grinding vehicle of the present invention consists essentially of varnishes cooked from hard resins and polyesters of polyhydric alcohols containing five to ten hydroxyl groups in which not less than one and not more than two of the hydroxyl groups of the polyhydric alcohol are esterified with a polyunsaturated water-insoluble fatty acid (i. e. drying oil fatty acids). The polyester oils are substantially non-drying, but will dry in the presence of other drying and semi-drying oils. Thus the varnish vehicles made from such oils will not skin or dry of themselves, but when incorporated into other drying or semi-drying vehicles, they do not deter the drying of these other vehicles. In this respect, therefore, these novel varnish vehicles are ideal grinding media for pigments.

The oils used in the grinding vehicle varnishes can be defined as synthetic polyester oils obtained by substantially completely esterifying polyhydric alcohols with at least two different acids. The polyesters have the general formula

30



where R is a residue of a polyhydric alcohol containing 5 to 10 hydroxyl groups, for instance, using dipentaerythritol the residue would have formula

35



Likewise, X represents an acid radical of a water-soluble monocarboxylic aliphatic acid containing at least two carbon atoms, e. g. the acetate radical; Y represents either an acid radical of a water-soluble monocarboxylic acid containing at least two carbon atoms (i. e. same as X), or Y can be a monocarboxylic acid containing an aromatic nucleus which constitutes at least about 50 per cent by weight of the molecule, e. g. benzoate or phenylacetate; Z represents an acid radical of poly-unsaturated fatty acid containing 10 or more carbon atoms or mixtures of these (i. e. a drying oil fatty acid or mixtures of the acids obtained by hydrolyzing a drying oil); x, y and z represent the number of moles of X, Y and Z groups respectively, neither x nor y being

40

45

50

55

less than  $\frac{1}{2}$  the number of hydroxyl groups in the polyhydric alcohol and  $z$  being not less than 1 nor more than 2; and where, in the polyester molecule as a whole, the total number of acid radicals is substantially equal to the number of hydroxyl groups in the polyhydric alcohol.

The polyester oils used in the invention are formed by esterifying a polyhydric alcohol containing five to ten hydroxyl groups with from about 1 to 2 mols of polyunsaturated water-insoluble acid, and the remaining hydroxyl groups with at least one acid of the group including water-soluble fatty acids and acids containing an aromatic nucleus in the molecule. Examples of water-insoluble polyunsaturated fatty acids include: sorbic acid, eleostearic acid, linoleic acid, and the like, or mixtures of such acids, for instance, dehydrated castor oil fatty acids, linseed oil fatty acids, soya oil fatty acids, fish oil fatty acids and the like, which may contain some water-insoluble saturated and monounsaturated acids.

Water-soluble fatty acids that may be used include acetic acid, propionic acid, butyric acid, isobutyric acid, and substitution products of these in which the substituent is unreactive during the process of preparing the polyesters, e. g. chloro acetic acid. Also other water-soluble acids such as levulinic acid are operable.

Monocarboxylic acids of the group containing an aromatic nucleus that are preferred contain only one aromatic nucleus in the molecule, such as, benzoic acid, toluic acids, phenylacetic acid, phenoxyacetic acid and the like. The aromatic nucleus should constitute at least about 50 per cent by weight of the molecule in order that the aromatic nature of the acid can be imparted to the polyester. Also, substitution products of these acids (e. g. mono and polychlorobenzoic acids) can be used provided that the substituent groups are unreactive during the preparation of esters. For this reason the use of acids containing nitro groups is not desirable.

The preparation of the polyesters used in the present invention can be accomplished by any of the usual methods of preparing esters, as by heating the reactants to a suitable temperature in the presence or absence of esterification catalysts.

The grinding vehicle varnishes made in accordance with the invention may be used alone, but preferably they are cut to not less than 75% total non-volatile content with a relatively high boiling hydrocarbon solvent. In this manner the viscosity of the vehicle is conveniently regulated. For most grinding procedures a viscosity of one to about five poises will be desired.

Due to the drying properties of the novel polyesters, when they are used in the presence of other drying vehicles, they do not show tackiness in air dried or baked films. Furthermore, the grinding vehicles made from these polyesters, being substantially non-drying alone, give pigment pastes that are free from skinning.

Also, the grinding vehicles of the present invention are non-reactive with pigments and have good wetting properties. For the best wetting properties the vehicle should be prepared from a polyester oil having an acid number of the order of 1 to 10.

The manner in which the vehicles are prepared from the polyester oils and the hard resins is in general analogous to the cooking of any other oleoresinous varnish. Since, for grinding purposes a rather low viscosity is required, it is necessary that the varnish vehicle be medium to long in oil length. Depending for the most part

upon the particular resin and polyester oil used, the varnishes should preferably be from about 15 to about 45 gallon oil length.

Of the hard resins, e. g. copal, Congo, kauri, phenolic resin, amber, rosin, limed rosin, ester gum, maleated rosin esters, and other modified rosin derivatives, commonly used in cooking oleoresinous varnishes, the maleated rosin esters containing 8 to 12% of maleic modification and having melting points of the order of 130-170° C. (Hercules drop method) are preferred.

The manner of practicing the invention will be more fully understood from the following examples in which the parts are by weight unless otherwise stated.

#### Example I

A mixture of 31.9 parts of soy fatty acids, 9.2 parts of benzoic acid and 20.9 parts of sorbitol (commercial grade containing about 84% sorbitol) was heated to 230° C. until esterification was complete (about four hours). The resultant product was refluxed with 38 parts of acetic anhydride for about two hours and then the acetic acid and excess acetic anhydride was removed by vacuum distillation. The oil left as residue had an acid number of 1.2 and a viscosity of 3.7 poises. This oil was readily compatible with hard varnish resins.

#### Example II

Using the oil prepared in Example I a 25 gallon oil length varnish was prepared by heating it at 225° C. with about half of its weight of an 8-12% maleated rosin ester resin (melting point, Hercules drop method, 130-140° C.). This varnish was then cut to 80% non-volatile content with high flash petroleum naphtha (boiling point 165-175° C.) to give a grinding vehicle of acid value 4.3 and a viscosity of 4.3 poises. The varnish was then used to make pigment pastes by dispersing an appropriate amount of the desired pigment in the varnish vehicle in conventional manner as by grinding on a 3-roll mill. These pigment pastes could then be incorporated in various types of vehicles to give coating compositions having properties equal to or better than similar compositions prepared from pigment pastes containing the various specific grinding vehicles for each type of composition that have been used heretofore.

Typical pigment paste compositions prepared using the varnish vehicle of Example II are:

|                   | Parts |
|-------------------|-------|
| A. Ferrite yellow | 60    |
| Vehicle           | 40    |
| B. Chrome green   | 50    |
| Vehicle           | 50    |

The pigment was dispersed in each instance by grinding in a three-roll mill. These pigment pastes showed no livering and no skinning at 158° F. for 120 hours.

As a test for the pigment pastes prepared using the grinding vehicle described above, the pigment pastes were dispersed in several vehicles which was thought to provide the severest test for the pastes. For this purpose a pure phenolic spar varnish was taken as an example of an oleoresinous varnish; a relatively short oil (29% soya fatty acids) modified phthalic alkyd and a phenolic modified alkyd were used as typical alkyds; and a straight run gum (kauri) nitrocellulose lacquer was used as a test lacquer. Although these formulations do not cover the broad field of coating formulations thoroughly it was believed that

since these particular ones had proved most difficult in obtaining compatibility between pigment paste and base vehicle that they would furnish the severest test for the grinding vehicle prepared in Example II. In the test the formulations were the same except for the grinding vehicle used to make the pigment pastes. Formulations containing each of the above vehicles and pigment paste prepared according to Example II were prepared and the vehicle of the paste was found to be satisfactorily compatible with each of the base vehicles. Also, upon comparing these four different formulations containing the same grinding vehicle with actual formulations of the same type containing a specific grinding vehicle in each formulation, it was found that test enamel formulations were equal or better in gloss and Sward hardness properties than the formulations used in actual practice and containing specific grinding vehicles for compatibility with each of the types of base vehicles. Thus the use of grinding vehicles prepared according to the present invention dispenses with the necessity of keeping numerous vehicles in stock, that is, a specific grinding vehicle for each type of formulation to be manufactured.

*Example III*

The polyester oil obtained in Example I was cooked into a 37.5 gallon varnish by heating it at 225° C. with one-third of its weight of an 8 to 12% maleated rosin ester resin. After reducing the varnish to 80% non-volatile content with high flash petroleum naphtha (boiling point 165-175° C.), the varnish was used as a grinding vehicle for making pigment pastes. The pigment pastes were tested in a manner similar to that used to test the pastes prepared from the Example II varnish and were found to give satisfactory compatibility, gloss and Sward hardness when used in oleoresinous, alkyd, and lacquer formulations.

*Example IV*

A polyester consisting of polypentaerythritol (commercial grade containing approximately 45 equal molecular amounts of di- and tripentaerythritol) esterified with approximately 1.5 moles of soya fatty acids, 1 mole of benzoic acid and 4.5 moles acetic acid was prepared by a procedure similar to that in Example I. For the purpose of calculating molar ratios of the molecular weight of polypentaerythritol was considered to be the average of the molecular weights of di- and tripentaerythritol. A 37.5 gallon varnish was prepared by heating this polypentaerythritol oil at 225° C. with one-third of its weight of an 8-12% maleated rosin ester resin (melting point, drop method, 130-140° C.). This varnish was then reduced to 80% non-volatile content with high flash petroleum naphtha (boiling point 165-175° C.) and used as a grinding vehicle in making pigment pastes. The pastes were readily dispersible in and compatible with oleoresinous, alkyd and lacquer formulations. Films of these final compositions formed on metal and air-dried or baked had good gloss and hardness.

*Example V*

The polyester oil of Example I was cooked into a varnish by heating it at 225° C. with one-third of its weight of an 8-12% maleated rosin ester resin (melting point, Hercules drop method, 152°-168° C.). The varnish was then cut to 80% non-volatile content and used as a grinding vehicle for preparing pigment pastes on a 3-roll

mill. The resulting pastes were suitably compatible with oleoresinous varnishes, alkyds and nitrocellulose lacquers. Enamels and lacquers prepared using the pastes had good air dry and baking properties and gave films having good adhesion, gloss and hardness.

Since numerous modifications of the invention can be practiced it is intended that the scope of the invention be limited only by the valid scope of the appended claims.

I claim:

1. A varnish vehicle suitable for use in grinding pigments for incorporation into oleoresinous varnishes, alkyds, lacquers, and the like, consisting essentially of not less than 75 parts of a 15 to 45 gallon length hard varnish resin-polyester oil varnish, the polyester oil comprising a substantially completely esterified polyhydric alcohol having the general formula



where R is a polyhydric alcohol residue of an alcohol containing 5 to 10 hydroxyl groups, X is an acid radical of a water-soluble monocarboxylic aliphatic acid containing at least two carbon atoms, Y is the acid radical of an acid of the group consisting of water-soluble monocarboxylic acids containing at least two carbon atoms and monocarboxylic acids containing a mononuclear aromatic ring, Z is an acid radical of polyunsaturated long chain fatty acid, and x, y and z equal the number of moles of X, Y and Z respectively, where neither x nor y is less than  $\frac{1}{10}$  the sum of x, y and z, and z is not less than 1 nor more than 2, and not more than 25 parts of a hydrocarbon solvent for the varnish.

2. A varnish vehicle suitable for use in grinding pigments for incorporation into oleoresinous varnishes, alkyds, lacquers and the like, consisting essentially of not less than 75 parts of a 15 to 45 gallon length maleated rosin ester resin-polyester oil varnish, the polyester oil comprising a substantially completely esterified polyhydric alcohol having the general formula



where R is a polyhydric alcohol residue of an alcohol containing 5 to 10 hydroxyl groups, X is an acid radical of a water-soluble monocarboxylic aliphatic acid containing at least two carbon atoms, Y is an acid radical of an acid of the group consisting of water-soluble monocarboxylic aliphatic acids containing at least two carbon atoms and monocarboxylic acids containing a mononuclear aromatic ring, Z is an acid radical of a polyunsaturated long chain fatty acid, and x, y and z equal the number of moles of X, Y and Z respectively, where neither x nor y is less than  $\frac{1}{10}$  the sum of x, y and z, and z is not less than 1 nor more than 2, and not more than 25 parts of a hydrocarbon solvent for the varnish.

3. A varnish vehicle suitable for use in grinding pigments for incorporation into oleoresinous varnishes, alkyds, lacquers and the like, consisting essentially of not less than 75 parts of a 15 to 45 gallon length maleated rosin ester resin-polyester oil varnish, the polyester oil comprising a substantially completely esterified polyhydric alcohol having the general formula



where R is a polyhydric alcohol residue of an alcohol containing 5 to 10 hydroxyl groups, X is

an acid radical of a water-soluble monocarboxylic aliphatic acid containing at least two carbon atoms, Y is the benzoate radical, Z is an acid radical of a polyunsaturated long chain fatty acid, and x, y and z equal the number of moles of X, Y and Z respectively, where neither x nor y is less than  $\frac{1}{10}$  the sum of x, y and z and z is not less than 1 nor more than 2, and not more than 25 parts of a hydrocarbon solvent for the varnish.

4. A varnish vehicle suitable for use in grinding 10 pigments for incorporation into oleoresinous varnishes, alkyds, lacquers and the like, consisting essentially of not less than 75 parts of a 15 to 45 gallon length maleated rosin ester resin-polyester oil varnish, the polyester oil comprising a substantially completely esterified polyhydric alcohol having the general formula



where R is a polyhydric alcohol residue of an alcohol containing 5 to 10 hydroxyl groups, X is the acetate radical, Y is the benzoate radical, Z is an acid radical of a polyunsaturated long chain fatty acid, and x, y and z equal the number of moles of X, Y and Z respectively, where neither x nor y is less than  $\frac{1}{10}$  the sum of x, y and z, and z is not less than 1 nor more than 2, and not more than 25 parts of a hydrocarbon solvent for the varnish.

5. A varnish vehicle suitable for use in grinding 15 pigments for incorporation into oleoresinous varnishes, alkyds, lacquers and the like, consisting essentially of not less than 75 parts of a 15 to 45 gallon length maleated rosin ester resin-polyester oil varnish, the polyester oil comprising a substantially completely esterified polyhydric alcohol having the general formula



where R is the residue of sorbitol, X is an acid radical of a water-soluble monocarboxylic aliphatic acid containing at least two carbon atoms, Y is an acid radical of an acid of the group consisting of water-soluble monocarboxylic aliphatic acids containing at least two carbon atoms and monocarboxylic acids containing a mononuclear aromatic ring, Z is an acid radical of the polyunsaturated long chain fatty acid, and x, y and z equal the number of moles of X, Y and Z respectively, where neither x nor y is less than  $\frac{1}{10}$  the sum of x, y and z, and z is not less than 1 nor more than 2, and not more than 25 parts of a hydrocarbon solvent for the varnish.

6. A varnish vehicle suitable for use in grinding 20 pigments for incorporation into oleoresinous varnishes, alkyds, lacquers and the like, consisting essentially of not less than 75 parts of a 15 to 45 gallon length maleated rosin ester resin-polyester oil varnish, the polyester oil comprising a substantially completely esterified polyhydric alcohol having the general formula



where R is the residue of sorbitol, X is the acetate radical, Y is the benzoate radical, Z is an acid radical of a polyunsaturated long chain fatty acid, and x, y and z equal the number of moles of X, Y and Z respectively, where neither x nor y is less than  $\frac{1}{10}$  the sum of x, y and z, and z is not less than 1 nor more than 2, and not more than 25 parts of a hydrocarbon solvent for the varnish.

7. A varnish vehicle suitable for use in grinding 25 pigments for incorporation into oleoresinous varnishes, alkyds, lacquers and the like, consisting essentially of not less than 75 parts of a 15 to 45 gallon length maleated rosin ester resin-polyester oil varnish, the polyester oil comprising a substantially completely esterified polyhydric alcohol having the general formula



where R is the residue of sorbitol, X is the acetate radical, Y is the benzoate radical, Z is the acid radical of soy fatty acid, and x, y and z equal the number of moles of X, Y and Z respectively, where neither x nor y is less than  $\frac{1}{10}$  the sum of x, y and z, and z is not less than 1 nor more than 2, and not more than 25 parts of a hydrocarbon solvent for the varnish.

8. A varnish vehicle suitable for use in grinding 30 pigments for incorporation into oleoresinous varnishes, alkyds, lacquers and the like, consisting essentially of not less than 75 parts of a 15 to 45 gallon length maleated rosin ester resin-polyester oil varnish, the polyester oil comprising a substantially completely esterified polyhydric alcohol having the general formula



35 where R is the residue of sorbitol, X is the acetate radical, Y is the phenoxyacetate radical, Z is the acid radical of soy fatty acid, and x, y and z equal the number of moles of X, Y and Z respectively, where neither x nor y is less than  $\frac{1}{10}$  the sum of x, y and z, and z is not less than 1 nor more than 2, and not more than 25 parts of a hydrocarbon solvent for the varnish.

9. A pigment paste suitable for incorporation 40 into oleoresinous varnishes, alkyds, lacquers, and the like, comprising a pigment dispersed in a vehicle consisting essentially of not less than 75 parts of a 15 to 45 gallon length hard varnish resin-polyester oil varnish, the polyester oil comprising a substantially completely esterified polyhydric alcohol having the general formula



45 where R is a polyhydric alcohol residue of an alcohol containing 5 to 10 hydroxyl groups, X is an acid radical of a water-soluble monocarboxylic aliphatic acid containing at least two carbon atoms, Y is the acid radical of an acid of the group consisting of water-soluble monocarboxylic acids containing at least two carbon atoms and monocarboxylic acids containing a mononuclear aromatic ring, Z is an acid radical of polyunsaturated long chain fatty acid, and x, y and z equal the number of moles of X, Y and Z respectively, where 50 neither x nor y is less than  $\frac{1}{10}$  of the sum of x, y and z, and z is not less than 1 nor more than 2, and not more than 25 parts of a hydrocarbon solvent for the varnish.

10. A pigment paste suitable for incorporation 55 into oleoresinous varnishes, alkyds, lacquers, and the like, comprising a pigment dispersed in a vehicle consisting essentially of not less than 75 parts of a 15 to 45 gallon length maleated rosin ester resin-polyester oil varnish, the polyester oil comprising a substantially completely esterified polyhydric alcohol having the general formula



75 where R is a polyhydric alcohol residue of an

alcohol containing 5 to 10 hydroxyl groups, X is an acid radical of a water-soluble monocarboxylic aliphatic acid containing at least two carbon atoms, Y is the acid radical of an acid of the group consisting of water-soluble monocarboxylic acids containing at least two carbon atoms and monocarboxylic acids containing a mono-nuclear aromatic ring, Z is an acid radical of polyunsaturated long chain fatty acid, and x, y and z equal the number of moles of X, Y and Z respectively, where neither x nor y is less than  $\frac{1}{10}$  the sum of x, y and z, and z is not less than 1 nor more than 2, and not more than 25 parts of a hydrocarbon solvent for the varnish.

11. A pigment paste suitable for incorporation into oleoresinous varnishes, alkyds, lacquers, and the like, comprising a pigment dispersed in a vehicle consisting essentially of not less than 75 parts of a 15 to 45 gallon length maleated rosin ester resin-polyester oil varnish, the polyester oil comprising a substantially completely esterified polyhydric alcohol having the general formula



where R is a polyhydric alcohol residue of an alcohol containing 5 to 10 hydroxyl groups, X is the acetate radical, Y is the benzoate radical, Z is an acid radical of a polyunsaturated long chain fatty acid, and x, y and z equal the number of moles of X and Y respectively, where neither x nor y is less than  $\frac{1}{10}$  the sum of x, y and z, and z is not less than 1 nor more than 2, and not more than 25

10

parts of a hydrocarbon solvent for the varnish.

12. A pigment paste suitable for incorporation into oleoresinous varnishes, alkyds, lacquers, and the like, comprising a pigment dispersed in a vehicle consisting essentially of not less than 75 parts of a 15 to 45 gallon length maleated rosin ester resin-polyester oil varnish, the polyester oil comprising a substantially completely esterified polyhydric alcohol having a general formula



where R is the residue of sorbitol, X is the acetate radical, Y is the benzoate radical, Z is an acid radical of a polyunsaturated long chain fatty acid, and x, y and z equal the number of moles of X, Y and Z respectively, where neither x nor y is less than  $\frac{1}{10}$  the sum of x, y and z, and z is not less than 1 nor more than 2, and not more than 25 parts of a hydrocarbon solvent for the varnish.

ZENO W. WICKS, JR.

#### REFERENCES CITED

The following references are of record in the file of this patent:

#### UNITED STATES PATENTS

| Number    | Name              | Date          |
|-----------|-------------------|---------------|
| 2,077,371 | Rheinekeet et al. | Apr. 13, 1937 |
| 2,390,202 | Burrell et al.    | Dec. 4, 1945  |

#### FOREIGN PATENTS

| Number  | Country       | Date          |
|---------|---------------|---------------|
| 452,138 | Great Britain | Aug. 10, 1936 |